

# UNITED STATES PATENT OFFICE.

CLARENCE I. B. HENNING, OF WILMINGTON, DELAWARE, ASSIGNOR TO E. I. DU PONT DE NEMOURS & COMPANY, OF WILMINGTON, DELAWARE, A CORPORATION OF DELAWARE.

## PROPELLENT POWDER AND PROCESS OF MAKING SAME.

1,336,463.

Specification of Letters Patent. Patented Apr. 13, 1920.

No Drawing.

Application filed August 23, 1919. Serial No. 319,485.

*To all whom it may concern:*

Be it known that I, CLARENCE I. B. HENNING, a citizen of the United States, and a resident of Wilmington, in the county of 5 New Castle and State of Delaware, have invented a certain new and useful Propellant Powder and Process of Making Same, of which the following is a specification.

This invention relates to propellant powder compositions containing constituents capable of counteracting metallic fouling, and to a process of making such compositions.

Metallic fouling of the bore of small arms 15 and ordnance, particularly military rifles and military guns, which is caused by the fusing of the metal from the projectile with the steel of the gun barrel, has for many years been a source of trouble.

It is well known that the introduction of breech loading in arms of all kinds subsequently led to giving rotation to the projectile by means of rifling with twists. As the chamber of the gun is larger than the 25 bore, the projectile is provided with a soft metal band, usually of copper. When the combustion of the propellant powder causes the projectile to move forward, the bands of the projectile which conform in shape to the 30 section of the rifling, assure the proper rotation to the projectile. As the band completely fills the cross section of the bore it also serves as a check to prevent the escape of gas past the projectile and in addition it 35 serves to center the projectile in the bore and to determine a fixed position of the projectile when rammed in the gun. During the passage of the projectile through the bore of the gun the copper from the band 40 fuses with the steel of the bore of the gun, due to the high temperature. This fouling of the bore of the gun is usually referred to as metallic fouling and the amount increases very rapidly as additional rounds 45 are fired in the gun and soon reaches a point where the accumulated metallic fouling seriously affects the accuracy of the gun and also reduces the diameter of the bore of the gun to a point where the continued use 50 of the gun is very dangerous because of developing too high pressure. It is, therefore, necessary after a relatively small num-

ber of rounds have been fired to either re-bore or re-line the gun.

In the case of small arms, as for example 55 military rifles, a very similar metallic fouling takes place, which is caused by the fusing of the cupro-nickel of the bullet with the steel of the bore of the rifle barrel. This metallic fouling very seriously affects 60 the accuracy of the rifle and necessitates constant cleaning with chemicals, usually referred to as doping, for the purpose of dissolving out the metallic fouling from the bore of the rifle.

This metallic fouling may be reduced to a certain extent by introducing into the cartridge or cartridge bag, together with the propellant charge, a small amount of metal in the form of foil or thin strips. The 70 metals which have given the most satisfactory results are tin, alloys of tin and lead, with or without the addition of zinc. The explanation of the removal of the metallic fouling in this way is that alloys of copper 75 and tin are extremely brittle at elevated temperatures and do not adhere to the bore of the gun as the copper does when fused with the steel in the absence of tin. When an alloy of tin and lead is used the alloy apparently breaks up at the time of combustion 80 of the propellant into two components, the tin uniting with the copper in the bore of the gun to form an alloy which is extremely brittle and does not adhere to the steel. 85 The lead apparently does not unite with the copper but acts simply as a lubricant for the succeeding rounds and tends to granulate the copper alloy and facilitate its removal.

Exhaustive tests have shown that the method of using an alloy of tin and lead in the manner above described is a very effective means of not only reducing the metallic fouling of the gun but also of removing metallic fouling already formed. This makes it possible to use the alloy only occasionally for the removal of metallic fouling whenever it has reached a very bad condition rather than to use the alloy continuously for keeping down the amount of metallic fouling.

There are a number of serious objections, however, to the above method of lessening

metallic fouling by adding a metal or an alloy to the propellant charge in the form of foil or thin strips. It is necessary to put the metal or alloy into separate packages 5 and add these to the cartridge or cartridge bags in the amount desired. This involves several additional operations in the preparation of the ammunition. Due to the carelessness of the workmen the metal may be 10 either entirely omitted from a charge or too much placed in the charge. The most important objection, however, is that the metal or alloy is not uniformly distributed throughout the propellant charge and consequently 15 the removal of the metallic fouling is not uniform throughout the bore of the gun.

I have discovered that if the metal or mixture of metals or alloy for reducing or 20 removing the metallic fouling be first finely powdered and then incorporated in the nitrocellulose or nitrocellulose-nitroglycerin colloid during the process of manufacture of the powder, a uniform distribution of the 25 metal or alloy throughout the powder will be insured and the use of this powder will be found to reduce the metallic fouling to one-third or one-fourth of the usual metallic fouling occurring when using powder 30 without addition of a metal or alloy. Furthermore, the smaller amount of metallic fouling which is formed in the bore of the rifle or gun will be found to be more uniformly distributed, in view of the fact that 35 the metal or alloy is uniformly distributed throughout the propellant powder. This more uniform distribution of the metallic fouling in the bore of the gun, taken with the smaller amount of metallic fouling formed, 40 decidedly improves the accuracy of the gun and increases its useful life.

The object of this improved method is not so much to reduce the metallic fouling already formed in the gun, which incidentally 45 can be accomplished by the use of powder of the composition herein set forth, but more especially to prevent as much as possible the occurrence of metallic fouling by having always present in the propellant 50 charge a small amount of metal or alloy uniformly distributed throughout the powder grains. In addition to the material reduction in the amount of metallic fouling it has been found that the muzzle flash is very 55 much reduced, caused by the cooling effect of the metal or alloy on the gases.

No difficulty in the manufacture of powder is caused by the additional step of incorporating finely powdered metal or alloy therein. The only requisite is to have the material powdered sufficiently fine to 60 pass readily through the steel wire screens used for screening the foreign particles from the nitrocellulose or nitrocellulose-nitroglycerin colloid made in the usual manner.

and also to pass readily through the dies used to form the powder strings prior to cutting into grains. The requisite fineness of the powdered metal or alloy will of course depend somewhat upon the size of 70 the powder to be made, but I have found, for example, that powdered tin which will pass through an 80-mesh screen is sufficiently fine for use in the usual sizes of rifle and cannon powders. It is obvious that 75 powdered tin finer than 80-mesh can be used. The amount of metal or alloy required to reduce the metallic fouling of the projectile depends upon a number of factors. In the case of the reduction of the 80 metallic fouling in the .30-cal. Springfield rifle by means of powdered tin, I have found that from about 2.5% to 5.0% of powdered tin gives very satisfactory results, depending on the kind of bullets and ballistic requirements. However, I do not care to limit 85 myself to the particular percentage of powdered tin or to any particular percentages or kinds of metals or mixture of metals or alloys, which I may desire to use because 90 it is obvious that I will use that amount and kind which may be readily ascertained by a test to give the best results for the particular use for which it is intended. For example, a suitable alloy of tin and lead is in 95 the proportion of 60% tin and 40% lead. However, the amount of tin can be very materially increased and the amount of lead decreased, if not entirely omitted, with very 100 satisfactory results.

My new process may be illustrated by the following example:—

The improved propellant powder, containing finely powdered metal, according to my invention, can be made by the usual process 105 for making propellant powder for small arms and ordnances. For example, sufficient wet nitrocellulose to give 100 parts by weight of nitrocellulose, which may be a mixture of nitrocellulose soluble in ether-alcohol with nitrocellulose relatively insoluble in ether-alcohol, or may be a soluble nitrocellulose alone, is dehydrated with ethyl alcohol of approximately 95% by volume or 190 proof, by means of a dehydrating press, in order to displace the water. The excess alcohol is removed from the nitrocellulose leaving about 33½ parts by 110 weight of alcohol in the dehydrated nitrocellulose. To this is added approximately 115 66⅔ parts by weight of ethyl-ether in a suitable mixing machine, preferably provided with brine refrigeration. To the nitrocellulose and solvent in the mixer there may be added one-half or more parts of diphenyl-amin or other stabilizer, with 1 to 5 or more parts of the powdered metal, such as powdered tin, together with other ingredients, if desired, such as graphite, nitro-compounds, etc. The composition is thoroughly 120 125 130

mixed and colloided, which operation in the mixer requires about  $\frac{1}{2}$  hour or more, depending on the efficiency of the mixer. After thorough mixing, the colloided composition is formed into preliminary blocks by means of a press. These blocks are then placed in a so-called finishing press, and the composition pressed through dies into strings, which strings are granulated by means of a cutting machine. The granulated powder is then placed for one or more days in solvent recovery apparatus to recover alcohol and ether, and then dried in water or air, to reduce the solvent remaining in the powder to a low amount. The powder is then air dried to remove excess surface moisture and may or may not be glazed.

Although tin and zinc, and the lead alloy of tin have been mentioned specifically above as suitable metals for incorporation in the powder to counteract metallic fouling, there may be used various other metals capable of forming with copper an alloy which is brittle at an elevated temperature.

My invention is, furthermore, not limited to powder capable of overcoming the metallic fouling in connection with projectiles having a soft metal band composed of copper, but is also applicable to cases in which the soft metal band comprises a substance other than copper either alone or in combination with copper. In any case whether the soft metal band consists entirely of copper or not, the powdered metal or metals incorporated in the powder should be capable of forming with the soft metal of the band an alloy brittle at an elevated temperature and not adhering as strongly to the bore of the gun as does the soft metal alone. For instance in small arms and munitions, the bullet is jacketed with an alloy of copper and nickel which according to usage in the United States is usually 85% copper and 15% nickel. My experiments indicate that tin incorporated in the powder is efficient in removing the fouling from this cupronickel alloy, as well as metallic copper fouling. This is particularly important because the majority of military small arms cartridges contain cupro-nickel jacket bullets.

I claim:

1. The process of producing a propellant powder capable of counteracting the metallic fouling of the bore of a gun ordinarily caused by soft metal carried by the projectile to be shot from said gun, which comprises incorporating in a propellant powder composition a finely sub-divided metal capable of forming with said soft metal an alloy which does not adhere as tenaciously to the bore of the gun at elevated temperatures as does the soft metal alone.

2. The process of producing a propellant powder capable of counteracting the metal-

lic fouling of the bore of a gun ordinarily caused by soft metal carried by the projectile to be shot from said gun, which comprises incorporating in a propellant powder composition a finely sub-divided metal capable of forming with said soft metal an alloy which is brittle at elevated temperatures.

3. The process of producing a propellant powder capable of counteracting the metallic fouling of the bore of a gun ordinarily caused by soft metal carried by the projectile to be shot from said gun, which comprises incorporating in a propellant powder composition a finely subdivided metallic substance comprising tin.

4. The process of producing a propellant powder capable of counteracting the metallic fouling of the bore of a gun ordinarily caused by soft metal carried by the projectile to be shot from said gun, which comprises incorporating in a propellant powder composition a finely subdivided metallic substance comprising tin and lead.

5. The process of producing nitrocellulose powder capable of counteracting the metallic fouling of the bore of a gun ordinarily caused by soft metal carried by the projectile to be shot from said gun, which comprises incorporating in a nitrocellulose powder composition during the step of colloiding the nitrocellulose a finely subdivided metal capable of forming with said soft metal an alloy which does not adhere as tenaciously to the bore of the gun at elevated temperatures as does the soft metal alone.

6. The process of producing nitrocellulose powder capable of counteracting the metallic fouling of the bore of a gun ordinarily caused by soft metal carried by the projectile to be shot from said gun, which comprises incorporating in a nitrocellulose powder composition during the step of colloiding the nitrocellulose a finely subdivided metal capable of forming with said soft metal an alloy which is brittle at elevated temperatures.

7. The process of producing nitrocellulose powder capable of counteracting the metallic fouling of the bore of a gun ordinarily caused by soft metal carried by the projectile to be shot from said gun, which comprises incorporating in a nitrocellulose powder composition during the step of colloiding the nitrocellulose a finely subdivided metallic substance comprising tin.

8. The process of producing nitrocellulose powder capable of counteracting the metallic fouling of the bore of a gun ordinarily caused by soft metal carried by the projectile to be shot from said gun, which comprises incorporating in a nitrocellulose powder composition during the step of colloiding the nitrocellulose a finely subdivided metallic substance comprising tin and lead.

9. A propellant powder containing in a finely subdivided condition a metal capable of reducing metallic fouling. 40
10. A propellant powder containing uniformly distributed therethrough in a finely subdivided condition a metal capable of reducing metallic fouling. 45
11. A propellant powder containing a finely subdivided metallic substance comprising tin uniformly distributed therethrough. 50
12. A propellant powder containing from about 1 to 5% of a finely subdivided metallic substance comprising tin uniformly distributed therethrough. 55
13. A propellant powder containing a finely subdivided metallic substance comprising tin and lead uniformly distributed therethrough. 60
- 20 14. A propellant powder containing from 1 to 5% of a finely subdivided metallic substance comprising tin and lead uniformly distributed therethrough. 65
- 25 15. A nitrocellulose explosive grain containing in a finely subdivided condition a metal capable of reducing metallic fouling. 70
- 30 16. A nitrocellulose explosive grain containing uniformly distributed therethrough in a finely subdivided condition a metal capable of reducing metallic fouling. 75
- 35 17. A nitrocellulose explosive grain containing a finely subdivided metallic substance comprising tin uniformly distributed therethrough. 80
- 40 18. A nitrocellulose explosive grain containing from about 1 to 5% of a finely subdivided metallic substance comprising tin uniformly distributed therethrough. 85
- 45 19. A nitrocellulose explosive grain containing a finely subdivided metallic substance comprising tin and lead uniformly distributed therethrough. 90
- 50 20. A nitrocellulose explosive grain containing from 1 to 5% of a finely subdivided metallic substance comprising tin and lead uniformly distributed therethrough. 95
- 55 21. A propellant powder containing a finely subdivided metallic substance comprising about three parts of tin to 2 parts of lead uniformly distributed therethrough. 100
- 60 22. A nitrocellulose explosive grain containing uniformly distributed therethrough a finely powdered metal capable of forming with the soft metal carried by a projectile which is to be propelled by the explosion of said grain, an alloy which is brittle at elevated temperatures. 105
- 65 23. A nitrocellulose explosive grain containing uniformly distributed therethrough a finely powdered metal capable of forming with copper an alloy which is brittle at elevated temperatures. 110
- 70 24. A nitrocellulose explosive grain containing uniformly distributed therethrough from about 1 to 5% of a finely powdered metal capable of forming with the soft metal carried by a projectile which is to be propelled by the explosion of said grain, an alloy which is brittle at elevated temperatures. 115
- 75 25. A nitrocellulose explosive grain containing uniformly distributed therethrough from about 1 to 5% of a finely powdered metal capable of forming with copper an alloy which is brittle at elevated temperatures. 120

In testimony whereof I affix my signature.  
CLARENCE I. B. HENNING.